

## UNITED STATES PATENT OFFICE.

MAX DRAEMANN, OF COLOGNE, GERMANY.

## MANUFACTURE OF RUBBER FILAMENTS OR THREADS.

No Drawing.

Application filed August 16, 1922. Serial No. 582,212.

*To all whom it may concern:*

Be it known that I, MAX DRAEMANN, citizen of Germany, residing at Cologne, Germany, have invented new and useful Improvements in or Relating to the Manufacture of Rubber Filaments or Threads, of which the following is a specification.

It has already been proposed to vulcanize a caoutchouc solution in a cold state with the aid of sulphureted hydrogen and sulphur dioxide by adding both gases consecutively to the caoutchouc after its solution in benzine. In this manner it is possible to vulcanize larger caoutchouc articles but the method above referred to is not suitable for the manufacture of thin rubber threads for the reason that at the moment in which the normal vulcanization is reached a contraction occurs, and it is then no longer possible to obtain smooth rubber filaments or threads of round cross section by squeezing the rubber solution from the squirting machine.

According to the present invention the above drawback is avoided by first treating the rubber solution with one of the vulcanizing gases, then moulding the filaments or threads to the action of the second vulcanizing gas. In this manner rubber filaments or threads of any desired length may be produced by performing the moulding stage between the reaction of the two complimentary vulcanizing gases. It is therefore possible according to the novel process to treat the caoutchouc solution for example first with sulphureted hydrogen or sulphur dioxide or some other vulcanizing gas, then to form from this gas-contained solution filaments or threads and finally to introduce the latter directly after their formation into a solution containing the complimentary gas for the sulphur formation. By appropriate manipulation the dissolving means is expelled whereupon the filaments or threads are reeled up and ready for further use. A practical length for the filaments or threads in this operation is about 300 to 500 metres.

Since in the case of rubber threads only very small cross sections come into question, it is desirable to perform the operation slowly. It is likewise of great importance that

the sulphur should be deposited very slowly in order that the filaments or threads may be uniform along their whole length both in regard of tearing-strength and ductility. This may be obtained by cooling the second gas, for example, in the case of sulphur dioxide a solution with benzine cooled down to about 5 to 10° C. may be employed; or the gas may be compressed until it is liquefied. The reaction of the two gases on the filaments or threads is then caused to take place in a retarded manner.

It has moreover been found that with the aid of the novel process individual filaments or threads immediately after their exit from the nozzles may be corded together shortly before, during or after the treatment with the second gas. The contraction of the substance forming the filaments or threads which takes place after this manipulation results in a sufficient strength to enable the filaments or threads to be subjected to further treatment. It is preferable to operate with very liquid solutions whereas generally speaking for manufacturing rubber threads only thick or viscous solutions can be employed, because the unvulcanized threads would at once deliquesce. By using highly liquid solutions the pressure on the caoutchouc mass may be considerably reduced or avoided. The advantage of corded resides in a greater strength of the filaments or threads produced.

Having now particularly described and ascertained the nature of my said invention and in what manner the same is to be performed, I declare that what I claim is:

1. A method for the manufacture of rubber filaments which consists in subjecting a rubber solution to the action of one of two complementary vulcanizing gases, forming the treated solution into thread-like filaments, and passing said filaments through a solution containing the other complementary gas.

2. A method for the manufacture of rubber filaments which consists in subjecting a rubber solution to the action of cooled sulphureted hydrogen, forming the treated solution into thread-like filaments, and then

subjecting said filaments to the action of sulphur dioxide.

3. A method for the manufacture of rubber filaments which consists in subjecting a rubber solution to the action of cooled sulphureted hydrogen, forming the treated solution into thread-like filaments, then sub-

jecting said filaments to the action of sulphur dioxide and cording the individual filaments together by means of a highly liquid <sup>10</sup> rubber solution.

In testimony whereof I have signed my name to this specification.

MAX DRAEMANN.